

# UNITED STATES PATENT OFFICE.

WILLIAM CARPENTER, OF CHARLOTTE, MICHIGAN.

## IMPROVEMENT IN WATER-PROOF PASTES.

Specification forming part of Letters Patent No. 149,440, dated April 7, 1874; application filed  
March 30, 1874.

*To all whom it may concern:*

Be it known that I, WILLIAM CARPENTER, of the town of Charlotte, in the county of Eaton, in the State of Michigan, have invented a certain Compound called Water-Proof Paste, for the purposes of wall-hangings, covering trunks and desks with leather, cloth, &c., engineering, book-binding, and other similar purposes, of which the following is a specification:

The nature of my invention consists of a solution of common glue in hot linseed-oil, to which is added starch, white lead, and shellac-varnish.

To compound this paste, melt over a gentle fire, or a water-bath, one pound of common glue with just enough linseed-oil to make a saturated solution of it, to which add a half pound of powdered clear-starch, stirring the mixture well during the operation to give it a

uniform consistency. Then add of best white lead half a pound, to render the composition water-proof and increase its durability; and, finally, to increase the adhesiveness of the paste and give it tone, pour in four ounces of fine shellac-varnish, and stir until the ingredients are reduced to a uniform mixture.

This paste is entirely water-proof, and effectually resists the action of time and moisture.

Having thus described my invention, what I claim as new is—

A composition consisting of glue, linseed-oil, white lead, shellac-varnish, and starch, in the proportions specified.

WILLIAM CARPENTER.

Witnesses:

SOLON C. KEMON,  
CHAS. A. PETTIT.